

## UNITED STATES PATENT OFFICE

2,432,056

PROCESS FOR CARROTTING FUR FOR  
FELTINGMilton Weissman, Rego Park, N. Y., assignor to  
A. Papish, Inc., Danbury, Conn., a corporation  
of ConnecticutNo Drawing. Application October 25, 1941,  
Serial No. 416,534

3 Claims. (Cl. 8—112)

1

The present invention relates to the processing of fur fibres preliminary to the felting operation thereof and it has for its object a process which will avoid the use of mercury nitrate which is customarily used with nitric acid in aqueous medium, and which employs a reagent combination inexpensive and certain in its action.

About the year 1725 the discovery was made that if, before removal from the pelt, the fur be brushed with a dilute solution of nitric acid and mercuric nitrate, very satisfactory felting properties are imparted to the fur. It is a treatment which has continued in use until the present day.

The most objectionable feature of the mercury carroting process is that it is highly toxic to the operating personnel engaged in the hatting industry. Therefore, a great deal of effort has been expended in an effort to discover a successful non-mercuric carrot.

The carroting process is usually accomplished by brushing the chemical carroting solution into the fur fibres while they are attached to the pelt. Other alternative methods sometimes used are—either spraying the fibres or total immersion thereof in the chemical solution; then the fur fibres are dried and subsequently removed from the pelt. Thereupon they are ready for the felting operation. In practice, however, carroted fur is generally stored for substantial periods of time before being utilized in the felting operations.

There are several non-mercuric carroting processes known today. However, the fact remains that mercury carrot is still preponderantly used in hat manufacture. The reason for this is that no heretofore known non-mercuric process can produce a fur which is the equal of mercury-carroted fur.

I have discovered that an excellent non-mercuric carroting solution is obtained by employing the sodium salt of polymerized or polycondensed dinaphthyl-methane-disulfonic acid in conjunction with an aqueous acidic mixture of hydrolyzing and oxidizing reagents.

As an example:

Per cent by weight

|                                                                                |      |
|--------------------------------------------------------------------------------|------|
| Sodium salt of polymerized or polycondensed dinaphthyl-methane-disulfonic acid | 2.0  |
| Nitric acid                                                                    | 5.0  |
| Hydrogen peroxide                                                              | 2.0  |
| Water                                                                          | 91.0 |

In the art various other acid hydrolyzing agents, including hydrochloric or sulfuric acid, and mixtures thereof, have been proposed and may be used in substitution of the nitric acid, when desired, and various substitutions for peroxide of hydrogen set forth in the art may likewise be employed, if desired.

Because of the different properties of the various types of fur fibres suitable for felting operations and because of the variations possible in

the drying conditions, those versed in the carroting art know that for any given set of operating conditions the proportions of the carroting solution can best be determined by test upon the particular fur fibres to be treated. It therefore is understood that the example is illustrative and that the proportions may vary in accordance with particular conditions. The solution may be combed into the fur while it is still on the pelts and after drying the fur may be cut from the pelts and used in the felting operation or aged by storing. I have found that the felting characteristic of the fur treated in accordance with my process is substantially improved. The carroted fur may be used with entire safety without any toxic effect. There is no discoloration of the fur so that white and light shades of fur fibres remain unchanged as to shade. Quick starting is a characteristic of my process and thus the felting operation is rapidly produced and manufacturing costs lowered.

Having described my invention, what I claim and desire to secure by Letters Patent is as follows:

1. A process for carroting fur for felting which consists in treating such fur fibres with a solution containing a sodium salt of condensed dinaphthyl-methane-disulfonic acid, a hydrolyzing agent and an oxidizing agent.
2. A process for carroting fur for felting which consists in treating such fur fibres with a solution containing a sodium salt of condensed dinaphthyl-methane-disulfonic acid, nitric acid and hydrogen peroxide.
3. A process for carroting fur for felting which consists in treating such fur fibres with a solution containing:

|                                                     | Per cent (approximately) |
|-----------------------------------------------------|--------------------------|
| A sodium salt of dinaphthyl-methane-disulfonic acid | 2                        |
| Nitric acid                                         | 5                        |
| Hydrogen peroxide                                   | 2                        |
| Water                                               | 91                       |

MILTON WEISSMAN.

## REFERENCES CITED

The following references are of record in the file of this patent:

## UNITED STATES PATENTS

| Number    | Name       | Date          |
|-----------|------------|---------------|
| 1,778,473 | Wagner     | Oct. 14, 1930 |
| 1,636,836 | Pott       | Oct. 9, 1928  |
| 2,169,997 | Fabian     | Aug. 22, 1939 |
| 1,885,887 | Beal       | Nov. 1, 1932  |
| 1,722,904 | Somerville | July 30, 1929 |
| 2,126,232 | Voss       | Aug. 9, 1938  |
| 1,616,103 | Baddiley   | Feb. 1, 1927  |
| 1,696,199 | Gunther    | Dec. 25, 1928 |

(Other references on following page)

| Number    | Name    | Date          |
|-----------|---------|---------------|
| 1,955,678 | Mercier | Apr. 17, 1934 |
| 2,179,371 | Dyer    | Nov. 7, 1939  |
| 2,029,322 | Jaeger  | Feb. 4, 1936  |

## FOREIGN PATENTS

| Number  | Country | Date          |
|---------|---------|---------------|
| 250,453 | Germany | Sept. 6, 1912 |
| 457,057 | Germany | Mar. 7, 1928  |

## OTHER REFERENCES

5 Weidlein, "Progress," News Edition of Industrial and Engineering Chemistry, April 20, 1932, page 99.

Beal et al., "Elimination of Mercury Hazard," News Edition, American Chemical Soc., Nov. 25, 1941, page 1234.